

Feb. 21, 1928.

1,659,897

J. SCHOENFELD

REFLECTOR FOR RADIANT HEATERS

Filed April 6, 1926

*Fig. 1.*



*Fig. 2.*



INVENTOR.

*Joseph Schoenfeld.*

BY *Dewey, Strong, Townsend & Lathus*  
ATTORNEYS.

## UNITED STATES PATENT OFFICE.

JOSEPH SCHOENFELD, OF ALAMEDA, CALIFORNIA, ASSIGNOR TO THE MAGNAVOX COMPANY, OF SAN FRANCISCO, CALIFORNIA, A CORPORATION OF ARIZONA.

## REFLECTOR FOR RADIANT HEATERS.

Application filed April 6, 1925. Serial No. 20,679.

This invention relates to reflector heaters, such as electric heaters and the like.

While electric heaters of the "reflector type" have been in more or less general use for a considerable number of years, commercially, they have not been as successful as other types of electric heaters since their general efficiency has been low. Such heaters are fairly efficient when the reflectors are new and bright, but the reflectors being subjected to the high temperature of the heating elements, become oxidized or tarnished and gradually lose their efficiency.

The object of the present invention is to generally improve and simplify the construction, operation and efficiency of reflectors of the character described, and particularly to provide a reflector for electric heaters which will not oxidize or tarnish when subjected to the high temperature of the heating elements or from atmospheric influences.

One form which my invention may assume is exemplified in the following description and illustrated in the accompanying drawings, in which—

Fig. 1 is a transverse vertical section of a radiant type of electric heater.

Fig. 2 is an enlarged cross-section of a portion of the reflector showing the manner in which it is coated to prevent oxidation.

Referring to the drawings in detail, and particularly to Fig. 1, A indicates in general an electric heater, the heater comprising a stand B upon which is mounted a reflector 2. Mounted within the reflector is an electric heat resistance element 3, which is maintained at a fairly high temperature when the heater is in use. The reflecting surface of heaters of this character is, as previously stated, subjected to the high temperature of the heating element and this heat causes oxidation and tarnishing of the reflecting surface. The reflector proper may have any cross-section or shape desired but it is preferably so designed that the majority of the heat and light rays radiating from the heating element will be reflected and projected in a forward direction. The most efficient surface of the reflector is that immediately adjacent the heating elements as this portion of the surface receives

the greatest amount of heat and light rays. This surface is also closest to the heating element and it is for this reason that it rapidly heats and oxidizes the metal. As the heater depends upon the reflecting efficiency of the reflector the efficiency drops as oxidation or tarnishing takes place.

The object of the present invention is to provide a reflecting surface which will not oxidize or tarnish due to the action of the heat produced by the resistance element or otherwise. This is accomplished in the following manner: The reflector proper may be constructed of any suitable metal; for instance, such as soft iron or steel. This is stamped or otherwise shaped between dies or the like and it is then annealed, pickled and otherwise cleaned to remove all traces of grease and dirt. The interior surface of the reflector which serves the function of reflecting and projecting the light and heat rays is then enamelled or glazed, this being accomplished by first spraying or otherwise applying a grounding coat thereon which contains silica or the like combined with a suitable fusing material so as to produce a more or less glazed surface when baked in an oven at a temperature of 1600° F. After the grounding coat has been applied, a glazing coat consisting of substantially the following composition is next applied, in approximately the following proportions:

70 barium carbonate, 180 borax, 500 flint, 500 feldspar, 70 soda ash, 70 saltpetre, 150 cryolite, 75 boric acid.

The reflector is again placed in the oven and subjected to a temperature of approximately 1400 to 1600° F. The two coatings of glazing material form a smooth, polished surface which is ideal for the reception of the final reflecting material or surface which is last applied. This material consists of a non-oxidizing metal, such as gold, which may be applied in the form of a chloride. This is permitted to thoroughly dry and the reflector is again fired in the oven at a temperature of approximately 1200° F., after which it is removed and cooled and thoroughly rinsed off with clean warm water, which will give the gold a bright lustre. The coating of gold may also be applied by electro-plating, but the best results have so

far been obtained by means of a chloride solution of approximately 10% strength, as a thin uniform film of gold may in this manner be applied.

- 5 A reflector constructed in this manner may be subjected to the high temperature of the electric resistance or heating element without tarnishing, as gold is not readily oxidized at temperatures less than 1800° F. In 10 actual practice, the temperature assumed seldom exceeds 600° F., due to the rapidity with which the heat is liberated by means of conduction, radiation, convection and otherwise, so the chance of oxidizing the gold 15 film is entirely eliminated. The temperature of the resistance or heating element proper seldom exceeds 1200° and it is for this reason that temperatures in excess of 600° F. are not exceeded in the reflector proper. 20 Gold has been specified as the material most suitable for the present purpose as it has proved an efficient reflector, both for the projection of the heat and the light rays. The projection of the light rays is not of 25 particular importance, but it is nevertheless desirable as it produces an optical effect to the extent that the entire surface of the reflector will appear as a glowing heated mass. Other non-oxidizing metals may be employed which will not oxidize when exposed 30 to the temperature specified, and I also wish it understood that the gold coating or film

may be applied to other materials or directly to the surface of the metal reflector. In some instances it might be desirable to construct the reflector proper of porcelain or other material. In that case the reflecting surface would not require glazing before applying the gold film or coating, as the porcelain is usually glazed during its manufacture.

Having thus described my invention, what I claim and desire to secure by Letters Patent is—

1. As an article of manufacture, a reflector for heaters comprising a body having a ground coat, a glazing coat united with the ground coat and consisting of barium carbonate, borax, flint, feldspar, soda ash, salt-petre, cryolite and boric acid, and a film of gold united with the glaze coat to provide a reflecting surface.
2. As an article of manufacture, a reflector for heaters comprising a body having a ground coat, a glaze coat united with the ground coat, and a thin film of gold united with the glaze coat.
3. As an article of manufacture, a reflector for heaters comprising a body having a ground coat consisting of silica combined with a fusing material, a glaze coat on the ground coat, and a thin film of gold on the glaze coat, the silica supporting the gold.

JOSEPH SCHOENFELD.